

April 3, 1956

J. S. SMART, JR

2,740,177

CONTINUOUS METAL CASTING PROCESS

Filed July 21, 1953

5 Sheets-Sheet 1



Fig:1.



Fig:6.



Fig:7.



Fig:8.

INVENTOR.  
JOHN S. SMART, JR.

BY *Edward J. Schaffner*

ATTORNEY

April 3, 1956

J. S. SMART, JR

2,740,177

CONTINUOUS METAL CASTING PROCESS

Filed July 21, 1953

5 Sheets-Sheet 2

Fig:2.



INVENTOR.

JOHN S. SMART, JR.

BY *Elwood J. Schaffer*

ATTORNEY

April 3, 1956

J. S. SMART, JR

2,740,177

CONTINUOUS METAL CASTING PROCESS

Filed July 21, 1953

5 Sheets-Sheet 3



Fig. 3.



Fig. 4.



Fig. 5.

INVENTOR.  
JOHN S. SMART, JR  
BY Elwood J. Schaffer

ATTORNEY

April 3, 1956

J. S. SMART, JR

2,740,177

CONTINUOUS METAL CASTING PROCESS

Filed July 21, 1953

5 Sheets-Sheet 4

*Fig:9.*



*Fig:10.*



*Fig:12.*



*Fig:11.*

INVENTOR.  
JOHN S. SMART, JR.  
BY *Elwood J. Schaffer*

ATTORNEY

April 3, 1956

J. S. SMART, JR

2,740,177

CONTINUOUS METAL CASTING PROCESS

Filed July 21, 1953

5 Sheets-Sheet 5



*Fig:13*



*Fig:14.*



*Fig:16.*



*Fig:15.*

INVENTOR.  
JOHN S. SMART, JR.

BY  
*Edward J. Schaffer*  
ATTORNEY

# United States Patent Office

2,740,177

Patented Apr. 3, 1956

1

2,740,177

## CONTINUOUS METAL CASTING PROCESS

John S. Smart, Jr., Westfield, N. J., assignor to American Smelting and Refining Company, New York, N. Y., a corporation of New Jersey

Application July 21, 1953, Serial No. 369,292

14 Claims. (Cl. 22—200.1)

This invention relates to a continuous metal casting process. More particularly, it relates to a process of this type in which an improved surface in the casting is produced. It especially relates to such a process in which an improved surface as well as other improved physical characteristics are produced in the casting.

Although many continuous casting processes have been proposed in the past, the castings from such prior processes have been characterized in varying degree by certain surface defects and internal faults. The surface defects in the castings from such prior processes may take the form of a plurality of small lateral surface cracks, wrinkles, crumpled areas which are usually composed of minute longitudinal gouges confined to an area or zone; or rough, shaggy surfaces. In some processes, the surface cracks may be so severe that the casting may break in the mold. Likewise, when casting alloys of non-eutectic and non-peritectic composition, the surface may become so rough and shaggy, due to bleeding of the lower freezing constituents, that the casting may become jammed in the mold and may be broken during the withdrawal from the mold.

In addition, dissolved gases released from the molten metal during the freezing may become entrapped in the interior of the casting and cause internal faults. Such entrapment generally results in a porous internal condition usually evidenced by small voids, generally ranging from visual to microscopic in size, and may cause brittleness in the casting or lowering of tensile strength. In some of the processes of the prior art the entrapment of the gases may result in relatively large interior voids, and this condition may become so severe as to cause a continuous channel in or adjacent the center of the casting. The art has long and diligently attempted to overcome the difficulties and disadvantages due to such surface defects and internal faults, but without success.

The principal object and advantage of the present invention resides in overcoming these difficulties of the prior art. These and other objects and advantages will become apparent from the following more detailed description of the invention.

Broadly, the invention comprehends introducing molten metal into one end of an open-ended mold having an uncooled section and a chill section of high thermal conductivity dividing the mold into an uncooled zone and a chill zone which is in substantially fixed relationship and immediately adjacent to the uncooled zone, with each of the zones surrounding the metal contained in their respective portions of the mold. During the casting the temperature of the inside surface of the uncooled zone is maintained above the melting point of the metal and the temperature of the inside surface of the chill zone is kept below the freezing point of the metal in that zone. The molten metal is introduced into the end of the mold containing the uncooled zone at a rate which, in relation to the rate of metal withdrawal from the mold, is sufficient to maintain molten, non-turbulent metal in the mold beyond that plane in the uncooled zone which lies

2

nearest the chill zone, and which passes through the entire cross-section of the mold intersecting the mold's longitudinal axis and in which the metal remains entirely molten during the process. The metal in the mold is maintained stationary with respect to the mold (i. e. no metal is withdrawn from the mold) until at least the outer surface of the metal in the chill zone extending substantially to said plane, is frozen into a shell of sufficient thickness and strength to permit intermittent withdrawal of the shell from the mold without rupture of the shell. During the formation of the shell, at least a major portion of the sensible and latent heat required to freeze the metal constituting the shell is rapidly withdrawn substantially laterally from the metal through the surface of the chill zone due to the high thermal conductivity of the walls of the mold in the chill zone. The frozen shell and any unfrozen metal encompassed thereby are withdrawn intermittently with respect to the mold from that end of the mold which contains the chill section by intermittently withdrawing the casting therefrom. The rate and period of the intermittent withdrawal of the casting is such that a major portion of the shell of the withdrawn casting is formed within the mold while the casting is stationary with respect thereto. The periods between withdrawal periods are also such that the metal remains entirely molten in the intersecting plane in the uncooled zone.

Withdrawing a major portion of the sensible and latent heat required to freeze the shell by a path which substantially parallels the longitudinal axis of the casting (as opposed to a path substantially lateral of this axis) results in a process which is too slow to be commercially acceptable. Moreover, in the casting of alloys of non-eutectic and non-peritectic composition, such procedure is too slow to prevent bleeding of lower melting constituents to the surface and their freezing thereon. In addition, the reduction or substantial elimination of surface cracks in the castings are not obtained in the absence in the process of any one of the other features set forth in the preceding paragraph. All of the features of the process stated in that paragraph are necessary, therefore, in the sense that they are critically important, in obtaining the present results as to smooth surface characteristics in a commercially acceptable process.

In casting alloys of non-eutectic and non-peritectic composition, (i. e., those whose liquidus and solidus temperatures do not coincide) and especially those having a wide range between their liquidus and solidus temperatures, it has been found that although the shell may be strong enough to withstand withdrawal from the mold, it nevertheless may contain interdendritic channels through which low melting constituents may bleed out to the surface of the casting by capillary action and freeze on the outer surface shell. The exudation and freezing of such low melting constituents, especially those which in the solid state are harder than the body of the casting, cause a rough, shaggy surface on the casting and may proceed to such an extent as to jam in the mold. In such an event, the casting may break due to the tension required to withdraw it, or the mold may break if it is constructed of a fairly brittle material such as graphite.

Such bleeding and the resulting rough, shaggy surface in castings of alloys of non-eutectic and non-peritectic composition are, as a practical matter, entirely eliminated by holding the metal stationary with respect to a mold having a chill section of high thermal conductivity and rapidly cooling the metal in the chill section until the temperature of at least the outer surface of the shell is below the freezing point of the lowest freezing component of the alloy which in the solid state is harder than the matrix of the casting. For best results this outer surface is cooled below the freezing point of the lowest freezing

component regardless of hardness. Rapid cooling to such temperature quickly freezes the metal in the interdendritic channels to produce a shell which is impervious to the low melting constituents before the latter material can bleed to the outer surface of the shell. Thereafter the outer surface of the shell is maintained below this temperature during the freezing of any remaining molten metal encompassed by the shell.

In conducting the process to obtain the improved results as to smooth surface and to reduce or eliminate roughness due to bleeding in the case of an alloy of non-eutectic and non-peritectic composition, the mold is preferably vertically disposed, with the uncooled zone in the upper portion and the chill zone in the lower portion of the mold. The most preferred procedure is to practice the process with a stationary mold and to withdraw the casting intermittently from the stationary mold. Another preferred feature is that the rate and period of the metal withdrawal from the mold is such that substantially all of the shell of the withdrawn metal is formed within the mold while the metal is stationary with respect thereto. The linear length of the withdrawal stroke preferably is not in excess of about 2". Withdrawal strokes not in excess of about 1" are the more preferred, with withdrawal strokes not in excess of about  $\frac{1}{2}$ " as the most preferred. Preferably also, the rate of withdrawal during the withdrawal stroke is as high as possible.

In conducting the process to obtain the additional benefit of reducing or avoiding gas entrapment in the casting, most of the above preferred features are necessary. Thus, it is necessary that the mold be vertically disposed with the uncooled zone above the chill zone to allow the released gas to escape upwardly and away from the freezing metal. Preferably, the mold is held stationary, i. e., stationary with respect to the earth, and the metal is withdrawn intermittently from the mold. It is also necessary, in order to obtain such benefit, that the linear length of the withdrawal stroke is not in excess of about 2" and that the period between any two adjacent withdrawal strokes, during which time the metal within the mold is stationary with respect thereto, is such that no metal in a molten state exists below the physical intersection between the uncooled section and the chill section at a distance which is greater than the largest lateral cross-sectional dimension of the mold cavity, and that molten metal only exists above the referred-to plane which intersects the longitudinal axis of the uncooled zone. Preferably, the withdrawal stroke does not exceed one linear inch and for best results the stroke is not in excess of about  $\frac{1}{2}$ ". Such a procedure insures the escape of the expelled gas by orderly progression and permits the gas to rise through the unfrozen metal.

The molten metal may be introduced into the mold in any desired manner. Thus, for example, the mold may be fixedly attached to the bottom of a molten metal holding furnace with the metal flowing directly into the mold so that a column of metal extends from the bottom of the casting to the top of the liquid metal in the holding furnace. Such introduction of the metal into the mold causes no turbulence in the molten metal in the mold. In such case, also, the metal has no free surface in the mold. Introduction of the metal so as to have a free metal surface in the mold, may also be practiced. For example, the metal may be led into the mold by a pipe or other conduit which terminates within the mold at, above or below the surface of the molten metal therein; or the metal may be introduced as a free falling stream.

The use of a free metal surface in the mold is preferred for casting shapes having a relatively large cross-sectional area, and especially solid shapes in which the smallest dimension of the cross-sectional area is greater than about 3". When using a free falling stream, it is important that the molten metal be introduced into the

mold at a rate sufficient, in relation to the rate of metal withdrawal from the mold, to insure the presence in the mold of a pool of molten metal above the solidifying metal in the mold and to maintain sufficient depth of metal in the pool to dampen the turbulence caused by the falling stream so as to establish a non-turbulent condition in the metal in the region in which the metal commences to freeze. If the pool of molten metal is too shallow in relation to the height of fall, the turbulence of the metal entering the mold may extend to the freezing metal and cause irregularities such as wrinkles, ripples, cold shuts and the like to be frozen into the surface of the casting. Although turbulent motion is to be avoided in this region, it should be noted that non-turbulent motion may exist and may in some instances be desirable.

The process may be practiced in connection with any ferrous or non-ferrous metal or alloy, and such material may be cast in any solid or hollow, circular or polygonal shape. The process of the invention is most effective in connection with the casting of copper and copper base alloys such as, for example, tough pitch copper, low oxygen coppers including oxygen-free copper and phosphorous deoxidized copper, brasses, bronzes and the

Excellent results are obtained with copper base alloys containing tin and those containing tin and lead. Heretofore, it has not been possible to cast such alloys in a continuous process without obtaining a rough and shaggy surface, and this has been especially true of copper base alloys containing at least 4% tin. With the present process, such alloys can be cast consistently with a smooth surface and with a smooth surface which is free of cracks by rapidly cooling the outer surface of the shell below the freezing point of the hard tin-rich constituents. Best surfaces, however, are obtained by rapid cooling below the freezing point of the lowest freezing constituent which, in the case of copper base alloys containing both lead and tin, is a soft lead-rich constituent, although with this latter procedure longer stationary periods are required. As used in this specification and the claims, alloys include metallic mixtures in which the components are completely miscible in each other in the molten phase, as well as metal mixtures which are not miscible in this phase.

The mold may be fabricated of any suitable material, and different materials may be used in any one mold. Material of high thermal conductivity is used to fabricate the chill section. Preferably, the surface of the uncooled section or this entire section is composed of a material which is, or is substantially, not wet or dissolved by the molten metal. In general, graphite molds are preferred, especially in the casting of copper or copper base alloys containing tin, although molds of a suitable metal may also be used.

When casting with a free metal surface in a graphite mold, the exposed interior and exterior walls of the uncooled section of the mold may be protected by a ceramic or replaceable graphite insert for this section. Instead of such an arrangement, this section may be protected by an inert or reducing material such as nitrogen, carbon monoxide or other reducing gas, powdered magnesia, powdered graphite, charcoal, coal, or coke breeze and the like. Alternatively also, the chill section may be composed of a metal, especially copper, and the uncooled section of graphite or a ceramic material. The chill zone may be established by a jacket surrounding the chill section of the mold through which water or any other fluid coolant may be circulated. The high thermal conductivity of the chill section thus affords rapid lateral extraction of heat from the metal in this portion of the mold. In the present invention, therefore, the mold is characterized in operation by cold walls in the chill section and a sharply increasing temperature gradient in the mold wall just above this section in the uncooled section.

The invention is further illustrated in the accompany-

ing drawings and examples. It should be understood, however, that the drawings and the examples are given for purposes of illustration and that the invention in its broader aspects is not limited thereto.

In the drawings:

Fig. 1 is an exaggerated view partly in vertical section illustrating a preferred method and apparatus for conducting the process of the invention to cast small shapes.

Fig. 2 is an exaggerated view partly in vertical section illustrating a preferred mode and apparatus for conducting the process to cast large shapes.

Fig. 3 is a vertical section through a mold and illustrates a modified method and mold for casting small shapes.

Fig. 4 is a top view of Fig. 3 along the line 4-4 in the direction of the arrows.

Fig. 5 is an enlarged vertical section of a mold illustrating the various conditions existing in the mold during the practice of the process.

Fig. 6 is a horizontal cross-section of the mold of Fig. 1.

Figs. 7 and 8 are similar to Fig. 6 and show molds of different cross-sectional shapes.

Fig. 9 is a specimen casting displaying surface cracks.

Fig. 10 is a specimen casting similar in composition to that of Fig. 9 but produced in accordance with the present process.

Fig. 11 is a specimen of an alloy of non-eutectic and non-peritectic composition displaying a rough, shaggy surface.

Fig. 12 is a specimen of an alloy of composition similar to that of Fig. 11 but cast in accordance with the present invention.

Fig. 13 is a specimen of metal displaying gas entrainment phenomena.

Fig. 14 is a specimen casting similar in composition to that of Fig. 13 but cast in accordance with the present process.

Fig. 15 is a disc which was cut from the specimen of Fig. 13 and then fractured. Before fracturing the disc it was partially severed by sawing along the line of fracture.

Fig. 16 is a disc similar to Fig. 15 but cut from the specimen of Fig. 14.

Referring to the drawings, in Fig. 1 there is shown a general assembly of a molten metal holding furnace 1, mold 2 and intermittent withdrawing means indicated generally by the numeral 3 for withdrawing casting 4 from the mold. The mold 2 extends through the bottom of the furnace 1 and in contact with the molten metal 5 therein. The mold is fixedly attached to the bottom of the furnace by means of threads 6 which engage mating threads 7 in the furnace bottom. The lower section of the mold is surrounded by water jacket 8 which preferably is fixedly attached thereto. Water or other coolant is circulated through the jacket in any desired manner.

The water jacket establishes in the mold an uncooled zone 9 and a chill zone 10. The latter zone extends vertically upward beyond the upper edge of the jacket 8 to the line C-C'. The exact location of this line and of the plane passing through it is determined by the thermal conductivity of the mold material, the thermal conductivity of the metal being cast, the sensible and latent heat of the metal to be cast, the cooling capacity of the jacket 8 in relation to the cross-sectional dimensions of the mold, the period during which the metal is stationary in the mold and the rate and period of the withdrawal stroke during the intermittent withdrawal. The plane passing through line C-C' is the lowest plane in which the metal remains entirely molten during the process.

The casting 4 is withdrawn intermittently from the mold by withdrawal means 3 which include rolls 11, at least one of which, as shown, may be driven by electric motor 12 by means of belt 13. Operatively connected to the motor 12 is starting and stopping switch 14 for operat-

ing the motor intermittently and thereby to cause the casting 4 to be withdrawn intermittently from the mold. The means 3 may also include any suitable braking means such as is illustrated by the shoe 15 which engages the brake drum 16 on the roll 11. The shoe may be operatively connected by levers 17 and 18 to switch 14 so as to brake and quickly stop the wheels when the motor 12 is turned off. The switch 14 may be manually operated or any suitable interval timer may be used which automatically makes and brakes the electrical supply to motor 12. More than one or all of the rolls 11 may be positively driven or positively braked. Any suitable withdrawal means may be used in place of that shown in the drawings. For best results, the withdrawal means is one which will start the rolls 11 at a relatively high speed so as to lower the casting 4 quickly during the intermittent withdrawal and to brake the downward motion of the casting when the motor 12 is turned off to obtain relatively prompt stoppage of the casting without undue coasting.

In conducting the process in apparatus of the type illustrated in Fig. 1, the level of molten metal in the holding furnace 1 is maintained above the upper edge 19 of the mold 2. As the casting 4 is withdrawn, the molten metal flows into the mold and the mold is thereby maintained filled with a column of metal. With this type of apparatus there is no free molten metal surface in the mold as the entire mold is filled with metal. Also, no turbulence exists in the molten metal in the mold such as would be the case if the metal were introduced as a free falling stream.

Fig. 2 shows a graphite mold in which the process may be conducted with a free metal surface in the mold, preferably for casting large shapes. As shown, the mold 2 is provided with water jacket 8 is supported by legs 20 which may be disposed in water tank 21 which may, in turn, rest on the foundation 22. Molten metal in the form of a free falling stream 23 is supplied to the mold by means of tilting furnace 24 and launder 25.

Any suitable tilting furnace may be used. As illustrated, the furnace may be pivotably mounted on support 27 and may be tilted as desired by hydraulic jack 28 suitably attached to the furnace at 29. The launder 25 likewise may be mounted on pivots 30 to adjust the height of the falling stream 23, which height preferably is as short as possible.

In operation, the furnace 24 is tilted to deliver molten metal at a rate which, in relation to the rate of withdrawal of the casting 4, maintains a pool of metal 31 in the mold 2 of sufficient depth to dampen the turbulence in the pool caused by the falling stream 23 so as to establish a non-turbulent condition in the molten metal in the bottom of the pool in the region above the curved line 32 below which the metal is in a frozen state.

The casting 4 may be withdrawn intermittently from the mold by rolls 11 in the same manner as described in Fig. 1. In passing to the rolls 11 the casting may pass through water tank 21 which may be provided with a suitable seal 33, such as a rubber gasket. Suitable severing mechanism (not shown) may be used in the apparatus of Figs. 1 and 2 below the rolls 11 to sever the casting into any desired length. Also, in starting either type of apparatus a solid bar may be placed in the rolls 11 so as to extend up into the mold. After the initially introduced metal has been frozen, the starting bar is withdrawn.

The apparatus illustrated in Fig. 2 is useful in casting large shapes and particularly for casting shapes of copper inasmuch as the length of the free falling stream may be controlled to minimize or control the amount of oxygen absorbed by the copper when it is poured through air. To minimize contact of the metal being cast with air or oxidizing gas, a layer of powdered material 34 may be maintained floating on the metal in the tilting furnace 24, the launder 25 and on the pool 31 in mold 2. It should be noted that protective material on the

pool 31 breaks the fall of the stream of metal 23 and therefore tends to reduce turbulence in the pool of metal 31. Accordingly, the minimum depth of the pool, to provide the desired quiescence in the bottom of the pool, may be correspondingly reduced. As used herein, a pool of metal of sufficient depth to establish the desired non-turbulence includes one in which a portion of the metal is replaced by a protective layer of solid material.

Where, due to the temperature of the molten metal, oxidation of the outside of the uncooled section of a graphite mold also presents a problem, this section may be protected by a wall 35 surrounding this portion of the mold. A space 36 between such a wall and the mold may also be filled with the protective material. Instead of the construction illustrated in Fig. 2, the uncooled section of the mold may contain a ceramic or a replaceable graphite insert protecting the inner or both the inner and outer surfaces of this section of the mold. The chill section also may be fabricated of a metal such as copper and the uncooled section of the mold, as well as the launder 25 and the space in furnace 24, may be protected by an inert or reducing gas. It should be noted that the construction of Fig. 2 affords good insulation and assures the maintenance of a temperature in the uncooled zone of the mold, which is above the melting point of the metal being cast. This is especially advantageous where the uncooled section of the mold is fabricated of a material of high thermal conductivity such as graphite. Heat, if and when necessary, may also be applied to this section of the mold.

Instead of conducting the process as illustrated in Figs. 1 and 2, in which the mold is stationary, the mold itself may be reciprocated so as to withdraw the casting intermittently with respect to the mold. Thus, for example, the casting may be lowered continuously with respect to a point in space and while being so lowered the mold may be lowered at the same speed as the casting during the period in which the metal is stationary with respect to the mold. The mold then is moved upwardly at the same or a different speed as the downward speed of the casting during the intermittent periods in which the metal is withdrawn from the mold. In such a procedure, as well as that described in Figs. 1 and 2, the relative motion between the mold and the casting during the intermittent withdrawal periods preferably is as rapid as practicable. Also at the end of the withdrawal stroke the relative motion is stopped as rapidly as possible with a minimum of coasting.

Regardless of the manner of accomplishing the intermittent removal of the casting, it has been found that the present process permits net withdrawal rates which are 20 to 30% greater than those possible with a process in which the casting is continuously withdrawn with respect to the mold. At the same time, all the enhanced surface and interior characteristics of the process are obtained.

In practicing the process to obtain an improved surface on the casting, the stationary period between any two adjacent withdrawal periods is of such duration as to form a shell of sufficient strength and thickness to withstand withdrawal of the casting without rupture. This condition is evidenced by the smooth appearance of the surface of the casting emerging from the mold, and in practice this period may be adjusted as required to obtain such surface characteristics. The shell thus formed extends substantially to the plane C—C' in Fig. 5.

Referring further to Fig. 5, as the metal freezes into the shell 37, illustrated by the cup-shape metal between the solid curved line passing through points C—E—C' and the solid curved line passing through points D—D', the metal begins to shrink. In a plane passing through the points D—D', the shell pulls away from the mold. Below this plane, the cooling effect of the chill section is reduced due to the poorer contact of the shell with the mold. Direct, and therefore highest, cooling contact between the mold and the casting exists in the area

C—D—D'—C' extending along the linear length C—D of the mold.

It is believed that one of the principal advantages of the invention resides in the fact that this area is as large and as sharply defined as possible. Under any particular set of conditions, a thermal balance between the uncooled and the chill sections of the mold is reached in a plane passing through the points C—C' above which all the metal is completely molten. Below a plane passing through points D—D', the metal does not directly contact the mold. The direct and rapid heat transfer over the enlarged area C—D—D'—C', while the metal is stationary with respect to the mold, results in the rapid formation of a shell 37 of which the portion extending substantially to the plane passing through points C—C' is of sufficient thickness and strength to withstand rupture upon withdrawal from the mold. It is further believed that this accounts for the twin benefits of enhanced surface characteristics and high net rate of casting withdrawal which are obtained by the process of the invention.

A major portion of the heat extracted during the freezing of the shell flows substantially laterally from the metal and laterally through the highly thermal conductive walls of the chill zone. When the shell 37 has become thick enough to permit withdrawal without rupture, a length of casting corresponding generally to the linear length of line C—D in Fig. 5, is withdrawn and the cycle is repeated. The rate of withdrawal is such that a major portion and preferably substantially all of the outer surface of the withdrawn casting is formed as shell 37 while the metal is stationary in the mold.

In conducting the process to obtain the enhanced surface characteristics only, the stationary period may be just sufficiently long to form a shell of required thickness to permit withdrawal which, in the case of alloys of non-eutectic and non peritectic composition, is also of sufficient duration to cool rapidly at least the outer surface portion of the shell to a temperature below the temperature of the lowest freezing component of the alloy which in the solid state is harder than the matrix of the casting. In such procedure, molten metal may exist in the interior of the casting to any desired depth below the edge of the chill section. The lowest level at which molten metal may exist in the interior of the casting with such a procedure will depend, among other factors, upon the size of the casting, the over-all length of the water jacket 8, the amount and extent of cooling below the plane passing through points D—D' in the mold, and the duration of the stationary period.

In the case of the stationary mold, the linear length of the withdrawal stroke is affected by the speed of withdrawal and especially the starting and stopping phases of this step, depending upon the mass of the casting. To obtain the enhanced surface characteristics, the withdrawal stroke preferably is not in excess of about 2" in length. Very good results are obtained with withdrawal strokes not in excess of about 1", and best results with withdrawal strokes not in excess of about 1/2". Also, to obtain the enhanced surface characteristics, the stationary period preferably is sufficiently long so that no molten metal exists in the casting below the intersection of the uncooled and the chill sections of the mold at a distance which is greater than the largest horizontal dimension of the mold cavity. This is illustrated in Fig. 1 by the point E'' below which no molten metal exists. The length of the line 38 extending from the top edge 39 of the water jacket 8 to the point E'' is not greater than the largest horizontal dimension of the mold cavity. This latter dimension is illustrated in Fig. 6 by the internal diameter 40 in the case of a mold cavity which is circular in cross-section. This dimension is also illustrated by the length 42 in the case of a rectangular mold cavity shown in Fig. 7 and by the line 43 in Fig. 8 in the case of a mold having a mandrel 44 for the casting of hollow shapes.

To obtain the enhanced surface characteristics and at the same time to prevent or reduce to a minimum the entrapment of gas in the interior of the casting, the preferred conditions set forth in the preceding paragraphs are necessary, as is also the feature that the mold must be vertically disposed with the uncooled zone above the chill zone. Within these limits, the shallowness of the unfrozen pool of metal below the plane passing through points C—C' (Fig. 5) may be controlled by controlling the duration of the stationary periods. The more shallow this pool becomes the less is the tendency for gas to become entrapped in the solidified casting. Substantially no gas is entrapped when the stationary period is such that the solidified metal extends to the curved line 41.

Instead of the mold shown in Figs. 1 and 2, a mold having a plurality of mold cavities may be used, especially in the casting of small shapes. Such alternative construction is illustrated in Figs. 3 and 4 in which the mold 2 is provided with a plurality of cavities 45, 46 and 47 with the chill zone being established by a single wafer jacket 8. With such a construction the plane passing through the points C—C', immediately above which all the metal in the mold remains entirely molten, does not lie in the horizontal plane. Also, when it is desired to obtain only the enhanced surface characteristics in the process, a horizontally disposed mold or a bottom-fed vertical mold with the uncooled section below the chill section may be used.

#### Example I

Commercially pure copper was cast in apparatus similar to that shown in Fig. 1 except that the casting was withdrawn continuously from the mold at a constant rate of  $9\frac{1}{4}$  inches per minute. A solid cylindrical casting 3 inches in diameter was produced. Circulating water was used in the water jacket 8 surrounding the graphite mold 2. Fig. 9 is a photolithograph of a section of the casting thus produced. It will be noted that the surface contains a plurality of horizontal cracks.

#### Example II

The procedure of Example I was repeated except that a solid, cylindrical casting 4 inches in diameter was produced and the casting was withdrawn intermittently from the stationary mold 2. The intermittent withdrawal periods were 3 seconds in duration, during each of which the linear length of casting withdrawn was  $\frac{1}{5}$  of an inch. Each stationary period between adjacent withdrawal periods was 1 second in duration. Fig. 10 is a photolithograph of the casting thus produced. It will be noted that the surface of the casting is smooth and free of surface cracks.

#### Example III

The procedure of Example I was repeated to produce a tube of an alloy composed of 88% copper, 10% tin, and 2% zinc. The tube produced was  $1\frac{1}{32}$  inches in outside diameter and  $\frac{1}{2}$  inch in its inside diameter. The graphite mold had the cross-section of that illustrated in Fig. 8. The water jacket surrounded the outside surface of the mold 2 in the chill section and no water was circulated through the mandrel 44. The tube was continuously withdrawn from the stationary mold at a constant rate of  $11\frac{1}{4}$  inches per minute. The surface of the tube thus produced is shown in Fig. 11. It will be noted that the surface is rough and shaggy in appearance. These rough and shaggy exudations were found to be composed of low melting, tin-rich constituents which were harder than the main body or matrix of the casting. Solid rods cast from the same alloy with similar casting procedure produced the same rough and shaggy surface.

#### Example IV

The procedure of Example I was repeated except that a solid, cylindrical casting  $1\frac{1}{8}$  inches in diameter was produced from an alloy similar to that of Example III containing 90% copper and 10% tin. In the present

example, however, the casting was withdrawn intermittently from the stationary mold. The intermittent withdrawal periods were 2 seconds in duration, and during each such period  $\frac{1}{6}$  linear inches of casting were withdrawn from the mold. Each stationary period between adjacent withdrawal periods was 2 seconds in duration. During the stationary periods the outer surface of the shell of the casting was rapidly reduced to a temperature well below the freezing temperature of the lowest freezing constituent in the alloy. The surface of the casting thus produced is shown in Fig. 12. It will be noted that it is free of the rough, shaggy exudations found in Fig. 11.

#### Example V

The procedure of Example I was again repeated to produce an alloy rod stock  $2\frac{1}{4}$  inches in diameter and composed of 90% copper, 5% tin and 5% lead. The rod was continuously withdrawn from the stationary mold at a constant rate of 6 inches per minute. Fig. 13 shows a cross-section of a broken specimen of the rod thus cast. The interior of the specimen was porous and also contained a continuous void at its center. Fig. 15 shows a wafer or disc cut from the rod and which was fractured by bending. It will be noted that the interior of the casting is porous. It was found that the central void extended the full length of the specimen.

#### Example VI

The procedure of Example I was repeated except that a solid, cylindrical casting  $2\frac{1}{4}$  inches in diameter and composed of 90% copper and 10% tin was produced by withdrawing the casting intermittently from the stationary mold. The intermittent withdrawal periods were 3 seconds in duration, and during each such period 0.35 linear inches of casting were withdrawn from the mold. Each stationary period between the withdrawal periods was 1 second in duration. During the stationary periods the surface of the outer shell of the rod was rapidly reduced to a temperature well below the freezing point of the lowest freezing constituent in the alloy. Under these conditions of casting, no molten metal exists in the casting at a point about one inch below the top of the water jacket. Referring to Fig. 1, the dimension of the line 38 is about one linear inch under the conditions of the present example. Fig. 14 shows a cross-section of a broken specimen of the rod thus cast. Fig. 16 shows a wafer cut from the rod and which was fractured by bending. It will be noted that the interior of the casting is free of porosity and displays a uniformly sound structure.

#### Example VII

The procedure of Example I was repeated to produce a rod stock  $1\frac{1}{4}$  inches in diameter analyzing 98% copper, 2% tin and 0.25% phosphorous. The rod was continuously withdrawn from the mold at the rate of  $5\frac{1}{2}$  inches per minute. The surface of the rod had the rough and shaggy surface illustrated in Fig. 11.

#### Example VIII

The same size and composition of rod as that set forth in Example VII was made in accordance with the present invention in apparatus of the type illustrated in Fig. 1 and using a graphite mold. The casting was withdrawn intermittently from the stationary mold using withdrawal periods of three seconds duration, during each of which 0.635 linear inches of casting were withdrawn. This amounted to a net withdrawal rate of  $9\frac{1}{2}$  inches per minute. The stationary periods were 1 second in duration. The surface of the outer shell of the rod was rapidly reduced during the stationary periods to a temperature well below the lowest freezing constituent in the alloy. The casting produced had a smooth, even surface similar to that illustrated in Fig. 12. The net withdrawal rate in this instance was 42% greater than that of Example VII.

## 11

## Example IX

The procedure of Example VII was repeated to produce rod stock 1½ inches in diameter and analyzing 84% copper, 10% tin, 2½% lead and 3½% nickel. The rod was withdrawn continuously from the stationary mold at a constant rate of 5½ inches per minute. The produced rod has a surface which was even more rough and shaggy than that of Example VII.

## Example X

The same size and composition of rod as that of Example IX was made in accordance with the present invention using apparatus of the type illustrated in Fig. 1 and which was equipped with a graphite mold. The casting was withdrawn intermittently from the stationary mold using withdrawal periods of three seconds duration. In each withdrawal period 0.465 linear inches of rod were withdrawn from the mold; this rate amounting to a net withdrawal speed of 7 inches per minute. The stationary periods were 1 second in duration. The outersurface of the shell of the rod formed in the mold was rapidly reduced during the stationary periods to a temperature well below the freezing point of the tin-rich constituents of the alloy but not below the freezing point of the lead-rich constituents. The casting had an exceptionally smooth, even surface of the type illustrated in Fig. 12.

In operating the process on a plant-size scale over a period of several months, cycles varying from a withdrawal period of one second and a stationary period of 4 seconds to a withdrawal period of 4 seconds and a stationary period of one second have been used with satisfactory results.

From the foregoing it will be seen that the present invention provides a continuous method of casting alloys of non-eutectic and non-peritectic composition to eliminate the rough surface caused by low melting components which in the solid state are harder than the body of the casting and which in prior processes bleed to and freeze on the surface of the casting. The invention also provides a method for casting metals and alloys so as to reduce or eliminate surface cracks. In addition, it provides a step for eliminating surface imperfections caused by turbulence in the molten metal immediately before freezing, such as is encountered with molds having a free metal surface into which molten metal is introduced as a free falling stream. The invention further provides a process in which castings are produced which have enhanced surface characteristics and at the same time improved internal characteristics by eliminating or reducing internal faults due to entrapment of gases which are released by the molten metal as it freezes.

What is claimed is:

1. A continuous metal casting process comprising introducing molten metal into one end of an open-ended mold having an uncooled section and a fixed cooled section of high thermal conductivity dividing the mold into an uncooled zone and a chill zone immediately adjacent to said uncooled zone with each of said zones surrounding the metal contained therein, continuously maintaining the temperature of the inside surface of said uncooled zone above the melting point and the temperature of the inside surface of said chill zone below the freezing point of the metal contained in the respective zones, said molten metal being introduced into the end of the mold containing the uncooled zone at a rate which in relation to the rate of cast metal withdrawn from the mold is sufficient to maintain molten and non-turbulent metal in the uncooled zone of the mold in the vicinity of a plane which intersects said zones, and in which plane the metal remains entirely molten, maintaining the metal stationary with respect to the mold in the chill zone until at least the outersurface of the metal extending substantially to said plane is frozen

- 5 into a shell of sufficient thickness and strength to overcome the surface friction forces between the mold and the shell to permit motion of the shell with respect to the mold without rupture of the shell, said shell being formed by withdrawing at least a major portion of the sensible and latent heat required to freeze said shell substantially laterally from the metal through the surface of said chill zone, thereafter withdrawing a predetermined length of cast metal from the other end of the 10 mold, stopping said cast metal withdrawal before shell formation takes place on a major portion of the outer-surface of the molten metal moving beyond said plane into said chill zone during said metal withdrawal, and repeating said shell freezing and said cast metal withdrawal steps until a casting of desired length is obtained, whereby a major proportion of the shell of the thus withdrawn metal is formed within the mold while stationary with respect thereto thereby enhancing the surface characteristics on the said withdrawn casting.
- 15 2. A continuous metal casting process comprising introducing molten metal into one end of an open-ended mold having an uncooled section and a fixed cooled section of high thermal conductivity dividing the mold into an uncooled zone and a chill zone immediately adjacent to said uncooled zone with each of said zones surrounding the metal contained therein, continuously maintaining the temperature of the inside surface of said uncooled zone above the melting point and the temperature of the inside surface of said chill zone below the freezing point of the metal contained in the respective zones, 20 said molten metal being introduced into the end of the mold containing the uncooled zone at a rate which in relation to the rate of cast metal withdrawn from the mold is sufficient to maintain molten and non-turbulent metal in the uncooled zone of the mold in the vicinity of a plane which intersects said zones and in which plane the metal remains entirely molten, maintaining the metal stationary with respect to the mold in the chill zone until at least the outersurface of the 25 metal extending substantially to said plane is frozen into a shell of sufficient thickness and strength to overcome the surface friction forces between the mold and the shell to permit rapid motion of the shell with respect to the mold without rupture of the shell, said shell being formed by withdrawing at least a major portion of the sensible and latent heat required to freeze said shell substantially laterally from the metal through the surface of said chill zone, thereafter rapidly withdrawing predetermined length of cast metal from the other end of the mold thereby rapidly moving molten metal beyond said plane into said chill zone substantially without shell formation on the moving outersurface thereof, stopping said metal withdrawal before substantial shell formation takes place on said moving outersurface, and repeating said stationary shell freezing step and said cast metal withdrawal step until a casting of desired length is obtained, whereby substantially all of the shell of the thus withdrawn metal is formed within the mold while stationary with respect thereto thereby obtaining a high net casting rate and a uniformly smooth surface free of surface cracks on the said withdrawn casting.
- 30 3. A process according to claim 2 in which said molten metal is introduced into the top of a vertically disposed mold having said uncooled zone in the upper portion and said chill zone in the lower portion thereof.
- 35 4. A process according to claim 3 in which said mold is maintained stationary during the process and the metal is withdrawn intermittently from the stationary mold.
- 40 5. A process according to claim 2 in which a free falling stream of molten metal is introduced into the top of a vertically disposed mold having said uncooled zone in the upper portion and said chill zone in the lower portion thereof, and in which there is maintained in the uncooled zone a pool of molten metal of sufficient depth to dampen
- 45 55 60 65 70 75

the turbulence caused by the incoming stream of metal and to establish non-turbulent metal in said vicinity of said plane.

6. A process according to claim 2 in which the molten metal introduced into said mold is an alloy of non-eutectic and non-peritectic composition, and said metal is held stationary with respect to the mold until the temperature of at least the outersurface of said shell is below the freezing point of the lowest freezing component of said alloy which in the solid state is harder than the body of the casting.

7. A process according to claim 6 in which the temperature of said outersurface of said shell is cooled below the freezing point of the lowest freezing component of said alloy.

8. A process according to claim 6 in which a copper base alloy is introduced into said mold, and the mold is a graphite mold.

9. A process according to claim 8 in which said alloy contains at least 4% tin.

10. A process according to claim 8 in which said alloy contains tin and lead, and in which said outersurface of said shell is cooled to a temperature below the freezing point of the lowest freezing component of said alloy.

11. A process according to claim 2 in which metal selected from the group consisting of copper and copper base alloys is cast and the mold is a graphite mold.

12. A process according to claim 11 in which an upright mold with an uncooled zone above the chill zone is used, free mold surface exists in the mold during the

10

15

20

25

casting procedure, and the exterior and exposed interior surfaces of the mold are protected from direct contact with air.

13. A process according to claim 2 in which a vertical mold having an uncooled zone above the chill zone is used, said mold is maintained stationary during the process, the length of the withdrawal stroke is not in excess of about two inches, and the stationary period between any two adjacent withdrawal periods is such that no metal in a molten condition exists below said plane at a distance which is greater than the largest horizontal dimension of the mold cavity thereby also reducing entrapment of gas in the freezing metal.

14. A process according to claim 13 in which said withdrawal strokes are not in excess of one-half inch.

References Cited in the file of this patent

UNITED STATES PATENTS

|           |                  |               |
|-----------|------------------|---------------|
| 2,128,943 | Hudson           | Sept. 6, 1938 |
| 2,136,394 | Poland et al.    | Nov. 15, 1938 |
| 2,195,809 | Betterton et al. | Apr. 2, 1940  |
| 2,225,416 | Junghans         | Dec. 17, 1940 |
| 2,242,350 | Eldred           | May 20, 1941  |
| 2,527,545 | Goss             | Oct. 31, 1950 |
| 2,667,673 | Harrison         | Feb. 2, 1954  |
| 2,682,691 | Harter           | July 6, 1954  |

FOREIGN PATENTS

|         |               |               |
|---------|---------------|---------------|
| 598,385 | Great Britain | Feb. 17, 1948 |
|---------|---------------|---------------|